

Feb. 12, 1952

G. BACKER

2,585,212

WOVEN FABRIC

Filed April 17, 1948



INVENTOR  
GEORGE BACKER

BY *Richard Feier*  
ATTORNEYS

## UNITED STATES PATENT OFFICE

2,585,212

## WOVEN FABRIC

George Backer, New York, N. Y.

Application April 17, 1948, Serial No. 21,701

1 Claim. (Cl. 139—420)

**1**

This invention relates to woven fabrics and refers more particularly to fabrics containing plastic threads.

An object of the present invention is the provision of a fabric which is ornamental and most effective in appearance and which has excellent durability and wear-resisting qualities.

Another object of the present invention is the provision of a woven fabric which can be conveniently utilized for curtains and table covers, and as a covering for various articles of furniture, including seats and cushions used in various vehicles.

A still further object of the present invention is to utilize the excellent qualities of vinylidene chloride for the manufacture of fabrics having an ornamental appearance and excellent wear resisting qualities.

Other objects of the present invention will become apparent in the course of the following specification.

The objects of the present invention may be realized through the provision of a woven fabric consisting of mixtures of synthetic and plastic threads.

In accordance with the preferred embodiment of the invention, the warp consists of a mixture of vinylidene chloride such as Saran in conjunction with rayon, acetate or cuprammonium rayon yarn while the filling consists solely of vinylidene chloride.

The invention will appear more clearly from the following detailed description when taken in connection with the accompanying drawing showing by way of example a preferred embodiment of the inventive idea.

The single figure of the drawing illustrates diagrammatically in a conventional manner the construction of a fabric of this invention.

The figure shows a warp consisting of a sequence of rayon threads 1 and vinylidene chloride threads 2 and a filling 3 consisting solely of vinylidene chloride threads.

The following are a number of examples of fabrics made in accordance with the principles of the present invention. These examples are given by way of illustration and it is obvious that various changes may be made in either the warp or the filling of the fabrics.

*Example 1*

The warp consists of vinylidene chloride threads and rayon threads. The vinylidene chloride thread has a diameter of 0.01" to 0.012" while the rayon thread has 900 deniers to 1100 deniers and

**2**

may be natural or dyed. The warp has 40 ends of rayon to the inch and 20 ends of vinylidene chloride to the inch arranged in groups of 8 ends of rayon next to 4 ends of vinylidene chloride thread. The filling consists solely of a vinylidene chloride thread having a diameter of 0.01" to 0.012" and 34 to 44 picks per inch.

The weave may be a 4 x 4 twill weave with two in a shed.

The fabric may be made by two warp beams both drawn in a loom together and three or four shuttles may be used. The warp is drawn in two in each heddle eye.

The fabric thus produced is subjected to a stiff sizing and is most suitable for dyeing. On the other hand, vinylidene chloride threads may have the required coloring incorporated therein at the time of the dyeing.

*Example 2*

The warp consists of vinylidene chloride threads as described above while the filling consists of a mixture of plastic and rayon threads, particularly of the type described in Example 1.

*Example 3*

Both warp and filling consist of mixtures of plastic and rayon threads, particularly of the type described in Example 1.

Furthermore, fabrics may be produced consisting of various mixtures of synthetic and plastic materials and warp and filling.

It was found that in a fabric made in accordance with the present invention, the advantageous qualities of vinylidene chloride are particularly enhanced by its use in the form of threads woven into a fabric. The fabric is quite light in weight and yet it is most suitable for use as an outer covering for articles of furniture, table covers or curtains. The fabric has excellent moisture resistance and takes a press easily.

The important characteristic feature of the fabric is that it has the strength and beauty of vinylidene chloride while avoiding the defects of this material. The fabric has low shrinkage characteristics and is most durable; it may have any suitable finish and be provided with a beautiful lustre.

Thus, a fabric made in accordance with the principles of the present invention has unusual properties and appearance and is particularly suitable for articles subjected to heavy wear, such as furniture coverings. The fabric may be pressed to a sharp crease yet will not muss or wrinkle at ordinary temperatures. Vinylidene

chloride used in the present invention consists, preferably, of extruded oriented supercooled strand material made by the Dow Chemical Company under the name Saran. It is apparent that the specific illustrations shown above have been given by way of illustration and not by way of limitation and that the fabrics above described are subjected to wide variation and modification without departing from the scope or intent of the present invention; all of which variations and modifications are to be included within the scope of the present invention.

What is claimed is:

A woven fabric, having a warp consisting of vinylidene chloride threads having a diameter of 0.01" to 0.012" and rayon threads of 900 to 1100 deniers, said warp having 8 ends of rayon

10 to 4 ends of vinylidene chloride threads as alternating groups of threads and a filling consisting of vinylidene chloride thread having a diameter of 0.01" to 0.012".

GEORGE BACKER.

#### REFERENCES CITED

The following references are of record in the file of this patent:

#### UNITED STATES PATENTS

| Number    | Name            | Date          |
|-----------|-----------------|---------------|
| 2,279,206 | Randall         | Apr. 7, 1942  |
| 2,312,089 | Gobeille        | Feb. 23, 1943 |
| 2,343,892 | Dodge et al.    | Mar. 14, 1944 |
| 2,353,090 | Shelmire et al. | July 4, 1944  |
| 2,433,722 | Weiss           | Dec. 30, 1947 |